

## UNITED STATES PATENT OFFICE

2,258,591

## LUBRICATING OIL COMPOSITION

Franz Rudolf Moser and Albert Johannes Dijksman, Amsterdam, Netherlands, assignors to Shell Development Company, San Francisco, Calif., a corporation of Delaware

No. Drawing. Application November 27, 1939,  
Serial No. 306,330. In the Netherlands December 5, 1938

1 Claim. (Cl. 252—35)

This invention deals with compounded mineral lubricating oils and, more particularly, deals with the addition of salts of aromatic monocarboxylic acids to mineral oils to produce lubricating oils of improved anti-corrosive properties for internal combustion engines, which oils have the property of preventing the sticking of piston rings when running these engines for long periods of time, and which have the ability to properly lubricate the cylinders and pistons under severe conditions of loading, i. e., which prevent cylinder abrasion.

It is known that in modern internal combustion engines, such as high speed Diesel engines, aviation gasoline engines, etc., which due to their high power output, operate at relatively high temperatures, piston rings have a tendency to become stuck in the grooves. Lacquer and/or carbon formation appear to be the principal reasons for this occurrence. The addition of small amounts of certain oil-soluble carboxylic acid salts, such as polyvalent metal salts of fatty acids and naphthenic acids, is known to reduce the ring sticking tendencies. The addition of small amounts of the foregoing salts or soaps, however, has one or more of the following disadvantages: The newer type bearings containing cadmium are corroded especially by the soaps of naphthenic and aliphatic acids. The soaps break down under the high temperatures obtained in lubrication and, thereupon, the oil loses its effectiveness. Certain of the above salts cause gelatinization in the lubricants, while others settle out of the lubricating oil during use.

Now, in accordance with our invention, we have found that polyvalent metal salts of aromatic monocarboxylic acids in which the carboxylic acid radical is directly attached to the ring and, more particularly, the basic salts of these acids when added to mineral oils in suitable quantities produce effective anti-ring sticking lubricants which are relatively free from the above disadvantages.

The salts of the aromatic acids employed may be those of mononuclear aromatic acids, such as benzoic acid, or polynuclear, such as naphthoic or anthracene carboxylic acid. These acids are all thermally very stable.

Especially valuable are polyvalent metal salts of the aromatic monocarboxylic acids and of these magnesium, calcium, strontium, barium, zinc, nickel, manganese, lead, copper, cobalt, and aluminum appear to be the most active.

To be effective as ring sticking inhibitors the salts should be soluble in the lubricating oil.

While many of the salts of these simple aromatic carboxylic acids are little soluble in mineral oils, similar salts of the corresponding alkylated acids are usually much more soluble. Thus, preferred acids contain one or several alkyl radicals, having preferably not more than six carbon atoms. Longer alkyl chains, though suitable from the point of view of enhancing solubility, tend to be thermally unstable. Examples of the solubilizing action of alkyl radicals are the following: Calcium naphthoate is practically insoluble in mineral lubricating oils, while the calcium salt of diethyl naphthoate is readily soluble.

Zinc benzoate dissolves in a furfural-refined Venezuelan distillate to the extent of about .03%. Methyl benzoate of zinc dissolves to about 1%. The solubility of the zinc salt of para-tertiary butyl benzoic acid is about 1.5% and that of di-tertiary butyl benzoic acid 2%.

If desired, the aromatic acids may also contain polar substitution radicals, i. e. radicals containing elements other than C and H, such as hydroxy, alkoxy, aroxy, hydrosulfide, amino, imino, halogen, etc., radicals. While, in general, these polar radicals raise the solubility to a lesser extent than alkyl radicals, and often depress, rather than enhance it, they frequently are advantageous in further reducing corrosiveness. The effect of halogen on solubility is illustrated by para-chlorbenzoic acid or para-brombenzoic acid, the zinc salts of which are soluble to the extent of about .5%. Very useful and comparatively easily prepared aromatic carboxylic acids are those prepared from alkyl phenols by the addition of CO<sub>2</sub> (Kolbe reaction). Alkyl phenols are obtainable by extraction of coal tar distillates or cracked petroleum distillates with aqueous alkali and acidification of the aqueous extract. An example of a salt of an acid of this type is the zinc salt of thymotinic acid which is quite soluble even in 100 V. I. lubricating oil and displays excellent anti-ring sticking properties.

Further, as an aid to solubility, we have found that if the salts are added to the lubricating oil at an elevated temperature in the range of 250° C. to 350° C., the dissolution of the salt in the oil is rendered much easier. Once they have been dissolved at elevated temperature, the solutions thus obtained tend to remain substantially stable also at normal temperature. The addition of high boiling oxygenated solvents, such as high boiling alcohols, esters, for example, butyl stearate, amyl ricinoleate, etc., may be added further to improve solubility and stability of solutions of the salts of this invention in lubricating oils.

Although we prefer to use about .5 to 1.5% of the salts in our lubricating oil, suitable amounts may be varied from approximately .2% to 2.5%. Amounts in excess of this limit tend to cause undue increase in viscosity as well as jelling of the oil.

Crankcase lubricating oils containing salts of monocarboxylic aromatic acids may also have present other compounding ingredients, such as oxidation inhibitors, pour-point depressors, 10 blooming agents and extreme pressure agents, preferably those containing at least one of the elements phosphorus, sulfur or chlorine.

The following examples further illustrate our invention:

About .8% by weight of the zinc salt of para-tertiary butyl benzoic acid was dissolved in a fur-fural-refined Venezuelan lubricating oil distillate at about 280° C. The resulting lubricating oil composition was found to be suitable for internal 20 lubrication of Diesel engines, materially retarding ring sticking and to have the advantage of

being very little corrosive to bearing metals containing cadmium.

About 1% by weight of the zinc salt of di-isopropyl salicylic acid was dissolved in a highly refined mineral lubricating oil at a temperature of about 200° C. When using the lubricating oil composition thus prepared in Diesel engines or aviation gasoline engines, piston ring sticking did not occur, whilst corrosion of bearing metals consisting of lead-bronze or cadmium-nickel was not observed.

Similar results were obtained when using the above-mentioned highly refined mineral oil, to which 1% by weight of the zinc salt of thymotinic acid had been added.

We claim as our invention:

A compounded mineral lubricating oil of improved anti-corrosive properties containing a small amount of the zinc salt of di-isopropyl salicylic acid.

FRANZ RUDOLF MOSER.  
ALBERT JOHANNES DIJKSMAN.